



US007670203B2

(12) **United States Patent**  
Gammel et al.

(10) Patent No.: US 7,670,203 B2  
(45) Date of Patent: Mar. 2, 2010

(54) **PROCESS FOR MAKING AN ON-CHIP VACUUM TUBE DEVICE**

(75) Inventors: **Peter Ledel Gammel**, Millburn, NJ (US); **Richard Edwin Howard**, Highland Park, NJ (US); **Omar Daniel Lopez**, Summit, NJ (US); **Wei Zhu**, Warren, NJ (US)

(73) Assignee: **Agere Systems Inc.**, Allentown, PA (US)

(\*) Notice: Subject to any disclaimer, the term of this patent is extended or adjusted under 35 U.S.C. 154(b) by 368 days.

(21) Appl. No.: 11/649,197

(22) Filed: **Jan. 3, 2007**

(65) **Prior Publication Data**

US 2007/0293115 A1 Dec. 20, 2007

### Related U.S. Application Data

(62) Division of application No. 09/651,696, filed on Aug. 30, 2000, now Pat. No. 7,259,510.

(51) **Int. Cl.**  
*H01J 9/02* (2006.01)  
*H01J 9/18* (2006.01)  
*H01J 1/02* (2006.01)

(52) U.S. Cl. .... 445/29; 445/23; 445/49;  
313/309; 313/495

(58) **Field of Classification Search** ..... 445/23–25,  
       445/49–51, 29, 1, 7, 33, 35, 46; 313/309,  
       313/336, 351, 146, 147, 149, 293–304, 495–497;  
       359/290, 291; 438/7–9, 57, 128–132, 454,  
       438/690, 759, 942, 943, 762; 216/11, 13,  
       216/40, 56

See application file for complete search history.

(56) **References Cited**

## U.S. PATENT DOCUMENTS

4,728,177 A 3/1988 Green

(Continued)

## FOREIGN PATENT DOCUMENTS

EP 880 077 A2 5/1998

(Continued)

## OTHER PUBLICATIONS

Fan et al., "Self-Oriented Regular Arrays of Carbon Nanotubes and Their Field Emission Properties", (1999), Science vol. 283, 512-514.\*

(Continued)

*Primary Examiner*—Bumsuk Won  
*Assistant Examiner*—Nathaniel J Lee

## ABSTRACT

A method of making a microelectromechanical microwave vacuum tube device is disclosed. The device is formed by defining structural regions and sacrificial regions in a substrate. The structural regions have flexural members. The substrate is treated to remove the sacrificial regions and release the structural regions such that the structural regions are moveable by the flexural members. The structural regions include a device cathode, a device grid or both a device cathode and a device grid. The cathode comprises electron emitters. The device further includes an output structure where amplified microwave power is removed from the device. In the method, the cathode surface and the grid surface are moved to a position where they are substantially parallel to each other and substantially perpendicular to the substrate. The device further comprises an anode that is substantially parallel to the cathode surface and the grid surface.

**24 Claims, 3 Drawing Sheets**



## U.S. PATENT DOCUMENTS

4,827,177 A 5/1989 Lee et al.  
 5,145,438 A \* 9/1992 Bol ..... 445/49  
 5,363,021 A 11/1994 MacDonald  
 5,386,172 A 1/1995 Komatsu  
 5,536,988 A 7/1996 Zhang et al.  
 5,637,539 A 6/1997 Hoffmann et al.  
 5,786,658 A 7/1998 Tsukamoto et al.  
 5,814,563 A \* 9/1998 Ding et al. ..... 438/714  
 5,912,094 A \* 6/1999 Aksyuk et al. ..... 430/5  
 5,955,828 A 9/1999 Sadwick et al.  
 6,000,981 A \* 12/1999 Knox et al. ..... 445/24  
 6,027,951 A 2/2000 MacDonald et al.  
 6,034,810 A 3/2000 Robinson et al.  
 6,046,840 A \* 4/2000 Huibers ..... 359/291  
 6,062,931 A \* 5/2000 Chuang et al. ..... 445/24  
 6,522,055 B2 2/2003 Uemura et al.  
 6,630,772 B1 \* 10/2003 Bower et al. ..... 313/311  
 6,686,680 B2 2/2004 Shaw et al.  
 6,803,725 B2 10/2004 Jin

## FOREIGN PATENT DOCUMENTS

EP 880077 A2 \* 11/1998  
 WO WO 9623229 A1 \* 8/1996  
 WO WO-98/44529 10/1998

## OTHER PUBLICATIONS

Qin et al., "Growing carbon nanotubes by microwave plasma enhanced chemical vapor deposition", (1998), Applied Physics Letters vol. 72, No. 26, 3437-3439.\*  
 Fan et al., "Self-Oriented Regular Arrays of Carbon Nanotubes and Their Field Emission Properties", (1999), Science vol. 282, 512-514.\*  
 Pister, Kristofer S.J., "Hinged Polysilicon Structures With Integrated CMOS TFTS", (1992), Proc. IEEE Solid State Sensor and Actuator Workshop, Hiltonhead, South Carolina, 136-139.\*  
 Ren et al., "Synthesis of Large Arrays of Well-Aligned Carbon Nanotubes on Glass", Science, vol. 282, 1105 (1998).

Fan et al., "Self-Oriented Regular Arrays of Carbon Nanotubes and Their Field Emission Properties", *Science* vol. 283, 512 (1999).  
 Rinzler et al., "Unraveling Nanotubes: Field Emission from an Atomic Wire", *Science*, vol. 269, 1550 (1995).  
 de Heer, et al., "A Carbon Nanotube Field-Emission Electron Source", *Science*, vol. 270, 1179 (1995).  
 Saito et al., "Cathode Ray Tube Lighting Elements with Carbon Nanotube Field Emitters", *Jpn. J. Appl. Phys.*, vol. 37, L346 (1998).  
 Wang et al., "A nanotube-based field-emission flat panel display", *Appl. Phys. Lett.*, vol. 72, 2912 (1998).  
 Bonard et al., "Field emission from single-wall carbon nanotube films", *Appl. Phys. Lett.*, vol. 73, 918 (1998).  
 D.A. Koester, et al. MUMPS™ Design handbook, Rev. 5.0 (2000).  
 Iannazzo, S., "A Survey Of The Present Status Of Vacuum Microelectronics", *Solid-State Electronics*, vol. 36, No. 3, pp. 301-320, Mar. 1, 1993.  
 Green, R., et al., "Vacuum Integrated Circuits", *IEDM 85*, pp. 172-175.  
 A.S. Gilmour, Jr., *Microwave Tubes*, Artech House, pp. 191-313 (1986).  
 I. Brodie, et al., "Vacuum microelectronics", *Advances in Electronics and Electron Physics*, vol. 83 (1992).  
 Ren et al., *Science*, vol. 282, 1105 (1998).  
 Fan et al., *Science* vol. 283, 512 (1999).  
 Rinzler et al., *Science*, vol. 269, 1550 (1995).  
 De Heer et al., *Science*, vol. 270, 1179 (1995).  
 Saito et al., *Jpn. J. Appl. Phys. Lett.*, vol. 37, L346 (1998).  
 Wang et al., *Appl. Phys. Lett.*, vol. 72, 2912 (1998).  
 Bonard et al., *Appl. Phys. Lett.*, vol. 73, 918 (1998).  
 D.A. Koester, et al. MUMPs™ Design Handbook, Rev. 5.0.  
 D.K. Lynn, et al., "Thermionic Integrated Circuits: Electronics For Hostile Environments", *IEEE Transactions on Nuclear Science*, vol. NS-32, No. 6 (1985).  
 U.S. Appl. No. 09/236,966, filed Jan. 25, 1999.  
 U.S. Appl. No. 09/236,933, filed Jan. 25, 1999.  
 U.S. Appl. No. 09/296,572, filed Apr. 22, 1999.  
 U.S. Appl. No. 09/512,873, filed Feb. 25, 2000.  
 U.S. Appl. No. 09/376,457, filed Aug. 18, 1999.

\* cited by examiner

FIG. 1A



FIG. 1B



FIG. 1C



FIG. 2



**PROCESS FOR MAKING AN ON-CHIP  
VACUUM TUBE DEVICE**

**CROSS-REFERENCE TO RELATED  
APPLICATIONS**

This application is a divisional of U.S. application Ser. No. 09/651,696, filed on Aug. 30, 2000, now U.S. Pat. No. 7,259,510, the disclosure of which is incorporated herein by reference.

**BACKGROUND OF THE INVENTION**

**1. Field of the Invention**

The invention relates to microwave vacuum tube devices.

**2. Discussion of the Related Art**

Microwave vacuum tube devices, such as power amplifiers, are essential components of many modern microwave systems including telecommunications, radar, electronic warfare and navigation systems. While semiconductor microwave amplifiers are available, they generally lack the power capabilities required by most microwave systems. Microwave vacuum tube amplifiers, in contrast, can provide higher microwave power by orders of magnitude. The higher power levels of vacuum tube devices are the result of the fact that electrons can travel at a much higher velocity in a vacuum with much less energy losses than in a solid semiconductor material. The higher speed of electrons permits a use of the larger structure with the same transit time. A larger structure, in turn, permits a greater power output, often required for efficient operations.

Microwave tube devices typically operate by introducing a beam of electrons into a region where the beam interacts with an input signal, and deriving an output signal from the thus-modulated beam. See, e.g., A. S. Gilmour, Jr., *Microwave Tubes*, Artech House, 1986, 191-313. Microwave tube devices include gridded tubes (e.g., triodes, tetrodes, pentodes, and klystrodes), klystrons, traveling wave tubes, crossed-field amplifiers and gyrotrons. All these devices contain the basic components of a cathode structure, an interaction structure, and an output structure. (A grid is generally used in the cathode structure, to initiate emission from electron emitters, and the grid can also be used to modulate the electron emission to get a desired output. As used herein, grid indicates any structure that controls electron emission from the cathode, and the grid can have, for example, multiple apertures or a single aperture.)

These devices are typically formed by mechanical assembly of the individual components, e.g., aligning and securing the individual elements on a supporting structure. Unfortunately, such assembly is not efficient and cost-effective, and inevitably introduces some misalignment and asymmetry into the structure. Some attempts to address these problems have led to use of sacrificial layers in a rigid structure, i.e., a structure is rigidly built with layers or regions that are removed in order to expose or free the components of the device. See, e.g., U.S. Pat. No. 5,637,539 and I. Brodie and C. Spindt, "Vacuum microelectronics," *Advances in Electronics and Electron Physics*, Vol. 83 (1992). These rigid structures generally reflected an improvement, but still encountered formidable fabrication problems, such as alignment issues and parasitic effects. Thus, improved fabrication methods are desired.

Improvements in the emission source of such microwave tube devices are also desired. The usual source of electrons is a thermionic emission cathode, which is typically formed from tungsten that is either coated with barium or barium

oxide, or mixed with thorium oxide. Thermionic emission cathodes must be heated to temperatures around 1000° C. to produce sufficient thermionic electron emission current, e.g., on the order of amperes per square centimeter. The necessity of heating thermionic cathodes to such high temperatures creates several problems. For example, the heating limits the lifetime of the cathodes, introduces warm-up delays, requires bulky auxiliary equipment for cooling, and tends to interfere with high-speed modulation of emission in gridded tubes.

10 An attractive alternative is field emission at room temperature, which is possible using suitable cold cathode materials. Conventional cold cathode materials are typically made of Spindt-type cathodes formed from either metal (such as Mo) or semiconductor (such as Si), with sharp tips in nanometer sizes. (See I. Brodie and C. Spindt, *supra*.) Unfortunately, while useful emission characteristics have been demonstrated for these materials, the control voltage required for emission is relatively high (around 100 V) because of their high work functions, and this high voltage operation both increases the 15 damage incurred by the emitter tips and also requires a supply of significant power densities. In addition, fabrication is complicated and costly, particularly for uniform tips across a large area. Thus, vacuum microelectronic devices that incorporate Spindt cathodes tend to suffer from various drawbacks. As an 20 alternative cold cathode material, carbon nanotubes have recently emerged as a potentially useful emitter material. Nanotubes' high aspect ratio (>1,000) and small tip radii of curvature (~10 nm), coupled with their high mechanical 25 strength and chemical stability, make them particularly attractive as electron field emitters.

For these reasons, improved vacuum microelectronic device designs that avoid current problems are desired, particularly designs incorporating improved cold cathode electron emitters.

35

**SUMMARY OF THE INVENTION**

The invention relates to a unique design and fabrication process for microwave vacuum tube devices. The process of 40 the invention provides such devices on a smaller scale and with better control of size, spacing, symmetry, and other parameters than is generally possible with current techniques. The process involves providing a structure having numerous structural regions that constitute the elements of the ultimate 45 device, and numerous sacrificial regions. The structure is subjected to a treatment, e.g., an etch, to remove the sacrificial regions—referred to as a release step. A key feature of the invention is that one or more of the structural regions have flexural members that provide for movement of the regions upon such release. Specifically, the structural regions having these flexural members either move into place themselves, e.g., in a pop-up design, or, alternatively, become capable of 50 being physically moved into place, e.g., by movement (typically rotation) around a flexural member (typically a hinge mechanism). This movement puts the elements of the device into the appropriate configuration. All the components of the device are capable of having such flexural members, including, e.g., a cathode structure, an input structure, an interaction 55 structure, an output structure and/or a collection structure. And it is therefore possible for all the components of the device to be arranged using such flexural members, or for there to be some combination of structural regions with and without such members.

(Flexural member includes any structure that induces or 60 allows movement of a structural region into its desired configuration in the device. Pop-up indicates that the structural region is induced to move upon release, without the need for

external force. Hinge mechanism indicates one or more flexural members, e.g., a hinge, that allows the component to be moved, e.g., rotated, by applying external force. The cathode structure contains a cathode and one or more grids. The input structure is where the microwave signal to be amplified is introduced (in some configurations, the input structure is a grid of the cathode structure). The interaction structure is where the electron beam interacts with the microwave signal to be amplified. The output structure is where the amplified microwave power is removed. The collection structure is where the electron beam is collected after the amplified microwave power has been removed.)

In one embodiment, reflected in FIG. 1A, the release step provides a device substrate comprising a cathode electrode, a grid, and an anode, each being substantially planar with the device substrate surface and attached to the device substrate by a flexural member, e.g., a hinge mechanism. A mask is placed over portions of the device substrate such that the cathode electrode surface is exposed while other components on the device substrate are covered, and electron emitters are formed on the exposed cathode electrode surface. The mask is then removed, and the cathode, grid, and anode are rotated, around the flexural member, such that their surfaces are substantially parallel with each other. (Removal of the mask includes complete detachment from the substrate, as well as simply rotating an attached mask away from the device components.)

The resultant devices are on a scale not typically attainable by conventional techniques. For example, in conventional gridded tubes the cathode electrode and grid typically have surfaces greater than  $10^7 \mu\text{m}^2$ , whereas according to the invention, it is possible to form a cathode electrode and grid having surfaces of  $10^2$  to  $10^6 \mu\text{m}^2$ . Similarly, it is possible to attain extremely small cathode-grid spacings in the invention, e.g., as low as 3  $\mu\text{m}$ , typically less than 50  $\mu\text{m}$ , whereas current devices typically have a gap greater than 50  $\mu\text{m}$ . Devices of this size are not only useful for typical applications of microwave tubes, such as wireless base stations, but are also potentially useful in smaller-scale applications such as wireless handsets. While a particular anode configuration is reflected in the above embodiment, the formation techniques of the invention are applicable to a wide variety of gridded microwave tube types, including triodes, tetrodes, pentodes, and klystrodes, as well as other microwave tube devices having a variety of cathode, input, interaction, output, and collection structures. It is also possible to simultaneously form numerous devices on a single substrate, and to interconnect at least a portion of such devices to provide an integrated microwave circuit.

#### BRIEF DESCRIPTION OF THE DRAWINGS

FIGS. 1A to 1C illustrate fabrication steps according to an embodiment of the invention.

FIG. 2 shows an actual device substrate surface made according to an embodiment of the invention.

#### DETAILED DESCRIPTION OF THE INVENTION

In one embodiment, a gridded microwave tube is formed as follows. The principles used in the fabrication are those applicable to a variety of microelectromechanical systems (MEMS). Detailed fabrication information is available from, for example, the Design Handbook of MUMPs (Multi-User MEMS Processes), a commercial program designed for general purpose micromachining, available from Cronos Integrated Microsystems, Research Triangle Park, North Carolina.

A 100 mm diameter, n-type, (100) oriented silicon wafer, with a resistivity of 1 to 2 ohm-cm is used as the initial substrate. The surface of the wafer is heavily doped with phosphorus in a standard diffusion furnace, using POC1 as the dopant source. The dopant helps to reduce or prevent charge feed through to the substrate from electrostatic devices on the surface.

Next, a 600 nm low-stress LPCVD (low pressure chemical vapor deposition) silicon nitride layer is deposited on the wafers as an electrical isolation layer. This is followed by the deposition of a 500 nm LPCVD polysilicon film—Poly 0. (It is also possible to use single crystal silicon, which provides increased thermal efficiency due to its higher thermal conductivity.) Poly 0 is then patterned by conventional photolithography, e.g., coating the wafers with photoresist, exposing the photoresist with the appropriate mask, and developing the exposed photoresist to create a pattern, and etching the pattern into the underlying layer using an RIE (Reactive Ion Etch) system.

20 A 2.0  $\mu\text{m}$  phosphosilicate glass (PSG) sacrificial layer is then deposited by LPCVD and annealed at 1050° C. for 1 hour in argon. (Sacrificial indicates that the layer is not intended to be part of the final device structure, but is instead intended to be removed to leave the desired micromechanical structures. Materials other than PSG are possible.) This layer of PSG, known as First Oxide, is removed at the end of the process to free the first mechanical layer of polysilicon. The sacrificial layer is photolithographically patterned with a mask, e.g., a DIMPLES mask, as known in the art, and the pattern is then transferred into the sacrificial PSG layer by RIE. The nominal depth of the dimples is 750 nm.

The wafers are then lithographically patterned with a third mask layer—ANCHOR1. After etching ANCHOR1 to provide anchor holes to be filled by the first structural layer, that 35 first structural layer of polysilicon (Poly 1) is deposited at a thickness of 2.0  $\mu\text{m}$  and fills the anchor holes. A 200 nm layer of PSG is deposited over the polysilicon and the wafer is annealed at 1050° C. for 1 hour. The anneal dopes the polysilicon with phosphorus from the PSG layers both above and below it. The anneal also serves to significantly reduce the net stress in the Poly 1 layer. The Poly 1 (and its PSG masking layer) is lithographically patterned using a mask designed to form the first structural layer POLY1. The PSG layer is etched to produce a hard mask for the subsequent polysilicon etch. 45 The hard mask is more resistant to the polysilicon etch chemistry than the photoresist and ensures better transfer of the pattern into the polysilicon. After etching the polysilicon, the photoresist is stripped and the remaining oxide hard mask is removed by RIE.

50 After Poly 1 is etched, a second PSG layer (Second Oxide) is deposited and annealed. The Second Oxide is patterned using two different etch masks with different objectives. The POLY1\_POLY2\_VIA level provides for etch holes in the Second Oxide down to the Poly 1 layer. This provides a 55 mechanical and electrical connection between the Poly 1 and Poly 2 layers. The POLY1\_POLY2\_VIA layer is lithographically patterned and etched by RIE. The ANCHOR2 level is provided to etch both the First and Second Oxide layers in one step, thereby eliminating any misalignment between separately etched holes. More importantly, the ANCHOR2 etch eliminates the need to make a cut in First Oxide unrelated to anchoring a Poly 1 structure. The ANCHOR2 layer is lithographically patterned and etched by RIE in the same way as POLY1\_POLY2\_VIA.

60 The second structural layer, Poly 2, is then deposited (1.5  $\mu\text{m}$  thick) followed by the deposition of 200 nm of PSG. As with Poly 1, the thin PSG layer acts as both an etch mask and

dopant source for Poly 2. The wafer is annealed for one hour at 1050° C. to dope the polysilicon and reduce the residual film stress. The Poly 2 layer is lithographically patterned with a seventh mask (POLY2), and the PSG and polysilicon layers are etched by RIE using the same processing conditions as for Poly 1. The photoresist is then stripped and the masking oxide is removed.

The final deposited layer is a 0.5  $\mu\text{m}$  metal layer that provides for probing, bonding, and/or electrical routing and connection. The wafer is patterned lithographically with the eighth mask (METAL) and the metal is deposited and patterned using lift-off to provide a desired metal pattern. e.g., metal conductors.

Once the structural fabrication is completed, the release of the sacrificial regions is performed by immersing the chip in a bath of 49% HF (room temperature) for 1.5 to 2 minutes. This is followed by several minutes in DI water and then alcohol (to reduce stiction—i.e., the sticking of the structural members to the surrounding material) followed by at least 10 minutes in an oven at 150° C.

FIG. 1A shows a device structure subsequent to the above process steps, for a triode device configuration. On the surface of a device substrate 10, e.g., a silicon nitride surface on a silicon wafer, are formed a cathode electrode 12 attached to the device substrate 10 surface by a hinge mechanism 13 (formed by two hinges), a grid 14 attached to the device substrate 10 surface by a hinge mechanism 15, and an anode 16 attached to the device substrate 10 surface by a hinge mechanism 17. Also on the substrate 10 surface are contacts 18 electrically connected to the cathode electrode 12, grid 14, and anode 16. The contacts 18 and connective wiring are typically polysilicon coated with gold, although other materials are possible. Design of the connective wiring must take into account the subsequent rotation of the cathode electrode 12, grid 14, and anode 16, to avoid breakage and/or reliability problems. The substrate 10 also has three locking mechanisms 24, 26, 28, which secure the cathode 12, grid 14, and anode 16 in an upright position, as discussed below. A mask 20 is also attached to the substrate 10 by a hinge mechanism 21, e.g., made up of four hinges. The mask contains an opening 22 such that when the mask is rotated on its hinges to cover the other components of the device substrate surface, the cathode electrode 12 remains exposed. It is then possible to form the cathode emitter structure without forming emitters on any other portion of the device. The emitter structure is discussed in more detail below. All these components, including the hinges, are formed by a micromachining process such as discussed above.

FIG. 1B shows the structure of FIG. 1A, without the mask, after emitters 30 have been formed on the cathode electrode 12. The cathode electrode 12, with attached emitters 30, the grid 14, and the anode 16, are then mechanically rotated on their hinges, 13, 15, 17 and brought to an upright position—substantially perpendicular to the surface of the device substrate 10. The locking mechanisms 24, 26, 28 are then rotated on their hinges to secure the cathode electrode 12, grid 14, and anode 16 in these upright positions.

A cross-section of the resulting structure is shown in FIG. 1C, with the cathode electrode 12, the grid 14, and the anode 16 arranged such that their surfaces are substantially parallel to each other, and substantially perpendicular to the surface of the device substrate 10. Vacuum sealing and packaging of the structure are then performed by conventional techniques.

Other uses of flexural members are also possible, e.g., pop-up members that induce movement of the structural regions into the desired configuration, upon release, without

the need for external force. Combinations of pop-up and hinged mechanisms are similarly possible.

In operation, as discussed in Gilmour, *supra*, a weak microwave signal to be amplified is applied between the grid and the cathode. The signal applied to the grid controls the number of electrons drawn from the cathode. During the positive half of the microwave cycle, more electrons are drawn. During the negative half, fewer electrons are drawn. This modulated beam of electrons passes through the grid and goes to the anode. A small voltage on the grid controls a large amount of current. As this current passes through an external load, it produces a large voltage, and the gridded tube thereby provides gain. Because the spacing between the grid and the cathode can be controlled to be very close, a triode (or other gridded tube) made according to the invention is expected to be capable of operating at very high frequencies, of 5 GHz or more.

Variations of these device structures are also possible. For example, to reduce grid heating caused by electrons impacting the grid, it is possible to use a shadow grid placed directly on the cathode surface. The shadow grid is identical to the structure of the active grid, and covers or blocks the emitters directly underneath the active grid material, thereby preventing emitting electrons from impacting the grid. It is also possible to selectively form the emitters on the cathode substrate such that few or no emitters are located beneath the grid wires, such that emission takes place primarily through the grid apertures.

It is apparent that other gridded tube designs such as a tetrode (adding another grid between the control grid and the anode to eliminate grid current induced by changes in anode potential) and a klystrode (using a resonant cavity anode to couple the output power) are able to be constructed in a similar fashion. Numerous other designs are also possible, including pentodes, traveling wave tubes, klystrons, and even displays. Vertical or horizontal arrangement on a substrate is possible. It is also apparent that the technique of the invention facilitates formation of numerous devices simultaneously on a single chip, and/or integrated on a single chip to form part of a complex microwave circuit. The fabrication techniques of the invention are similarly able to provide more symmetrical and balanced components in a microwave system, which contribute to improved accuracy and noise control than conventional designs.

A variety of cold cathode emitter materials are possible, including carbon nanotubes, diamond, and amorphous carbon. Carbon nanotubes are particularly attractive as field emitters because their high aspect ratio (>1,000), one-dimensional structure, and small tip radii of curvature (~10 nm) tend to effectively concentrate the electric field. In addition, the atomic arrangement in a nanotube structure imparts superior mechanical strength and chemical stability, both of which make nanotube field emitters robust and stable. It is possible to prepare carbon nanotubes by a variety of techniques, including carbon-arc discharge, chemical vapor deposition via catalytic pyrolysis of hydrocarbons, laser ablation of a catalytic metal-containing graphite target, or condensed-phase electrolysis. Depending on the method of preparation and the specific process parameters, the nanotubes are produced multi-walled, single-walled, or as bundles of single-walled tubules, and can adopt various shapes such as straight, curved, planar-spiral and helix. Carbon nanotubes are typically grown in the form of randomly oriented, needle-like or spaghetti-like mats. However, oriented nanotube structures are also possible, as reflected in Ren et al., *Science*, Vol. 282, 1105, (1998); Fan et al., *Science*, Vol. 283, 512 (1999).

Carbon nanotube emitters are discussed, for example, in Rinzler et al., *Science*, Vol. 269, 1550 (1995); De Heer et al., *Science*, Vol. 270, 1179 (1995); Saito et al., *Jpn. J. Appl. Phys.*, Vol. 37, L346 (1998); Wang et al., *Appl. Phys. Lett.*, Vol. 70, 3308, (1997); Saito et al., *Jpn. J. Appl. Phys.*, Vol. 36, L1340 (1997); Wang et al. *Appl. Phys. Lett.*, Vol. 72, 2912 (1998); and Bonard et al., *Appl. Phys. Lett.*, Vol. 73, 918 (1998).

Techniques for forming nanotube field emitter structures, with both oriented and non-oriented nanotubes structures are also described in patent application Ser. Nos. 09/236,966, 09/236,933, 09/296,572, 09/351,537, 09/512,873, and 09/376,457, the disclosures of which are hereby incorporated by reference.

As reflected in these techniques, it is possible to form carbon nanotube emitters on a substrate by either in-situ growth or post-deposition spraying techniques. For in-situ growth in the invention, the device substrate, with mask in place over the components other than the cathode electrode surface, is generally placed in a chemical vapor deposition chamber, and pre-coated with a thin layer (e.g., 1-20 nm thick) of catalyst metal such as Co, Ni, or Fe (or formed from such a metal). The gas chemistry is typically hydrocarbon or carbon dioxide mixed with hydrogen or ammonia. Depending on specific process conditions, it is possible to grow the nanotubes in either an aligned or random manner. Optionally, a plasma enhanced chemical vapor deposition technique is used to grow highly aligned nanotubes on the substrate surface, as disclosed in co-assigned patent application Ser. No. 09/376,457, *supra*. Other techniques are also possible.

In a typical post-deposition technique, reflected, for example, in patent application Ser. No. 09/296,572, *supra*, pre-formed and purified nanotube powders are mixed with solvents and optionally binders (which are pyrolyzed later) to form a solution or slurry. The mixture is then disposed, e.g., dispersed by spray, onto the masked device substrate in which the cathode electrode surface is exposed. The cathode electrode optionally is provided with a layer of a carbon dissolving element (e.g., Ni, Fe, Co) or a carbide forming element (e.g., Si, Mo, Ti, Ta, Cr), to form a desired emitter structure. Annealing in either air, vacuum or inert atmosphere is followed to drive out the solvent, leaving a nanotube emitter structure on the substrate. And where the carbon dissolving or carbide forming elements are present, annealing promotes improved adhesion. Other post-deposition techniques are also possible.

The diameter of the field-emitting nanotubes is typically 1 to 300 nm. The length of the nanotubes is typically 0.05 to 100  $\mu\text{m}$ . To maintain the small gap between the cathode and the grid, and thereby achieve a reduced transit time and a higher operating frequency, the nanotubes advantageously exhibit a relatively uniform height, e.g., at least 90% of the nanotubes have a height that varies no more than 20% from the average height.

Because of the nanometer scale of the nanotubes, the nanotube emitters provide many potential emitting points, typically more than  $10^9$  emitting tips per square centimeter assuming a 10% area coverage and 10% activated emitters from 30 nm (in diameter) sized nanotubes. The emitter site density in the invention is typically at least  $10^3/\text{cm}^2$ , advantageously at least  $10^4/\text{cm}^2$  and more advantageously at least  $10^5/\text{cm}^2$ . The nanotube-containing cathode requires a turn-on field of less than  $2\text{ V}/\mu\text{m}$  to generate 1 nA of emission current, and exhibits an emission current density of at least  $0.1\text{ A}/\text{cm}^2$ , advantageously at least  $0.5\text{ A}/\text{cm}^2$ , at an electric field of 5 to  $50\text{ V}/\mu\text{m}$ .

## EXAMPLE

FIG. 2 shows a device substrate fabricated according to the invention. The device components were fabricated by the procedure presented above. The cathode, grid, and anode had surfaces  $100\text{ }\mu\text{m} \times 100\text{ }\mu\text{m}$ , and were  $2\text{ }\mu\text{m}$  thick. The apertures of the grid were  $6\text{ }\mu\text{m}$  across (in the direction parallel to the grid wires). The gap between the cathode and grid, when raised to a position perpendicular to the device substrate, was about  $40\text{ }\mu\text{m}$ .

Nanotube emitters were formed on the cathode electrode by a microwave plasma enhanced chemical vapor deposition technique. Specifically, after the mask was placed over the device substrate—leaving the cathode electrode surface exposed, an approximately 2 nm layer of cobalt was sputter-deposited through the opening onto the cathode electrode. The structure was then transferred in air to a microwave plasma enhanced chemical vapor deposition (MPECVD) system to start the nanotube growth. The structure was heated to 800° C. in flowing hydrogen in 10 minutes. A microwave plasma of ammonia ( $\text{NH}_3$ ) and 10 to 30 vol. % acetylene ( $\text{C}_2\text{H}_2$ ) was then ignited to start the nanotube growth. The growth process lasted about 2 minutes. The structure was then cooled to room temperature, again in flowing hydrogen. As shown in FIG. 2, the nanotubes grown under these conditions were aligned. Because the nanotube growth is highly selective, with growth occurring only in areas where cobalt is present, the nanotubes were substantially confined on the cathode in an area defined by the opening in the mask through which cobalt is deposited.

Other embodiments of the invention will be apparent to those skilled in the art from consideration of the specification and practice of the invention disclosed herein.

The invention claimed is:

1. A process for fabricating a vacuum microelectromechanical device, comprising:
  - providing a structure comprising a plurality of structural regions formed on and among a plurality of sacrificial regions, wherein a mask component having an opening therein is defined in one structural region and at least one device component is defined in a second structural region wherein the mask component and the at least one device component each comprise one or more flexural members;
  - treating the structure to remove the sacrificial regions, wherein the removal releases the structural regions comprising the mask component and the at least one device component such that the mask component and the at least one device component are moveable by a force exerted by the one or more flexural members or such that the mask component and the at least one device component become capable of being moved about the one or more flexural members, and wherein the at least one device component is a cathode structure comprising an electrode and wherein the released structural regions further comprises at least a portion of one or more other device components selected from the group consisting of an input structure, an interaction structure, an output structure, and a collection structure;
  - rotating the mask component to overlay the cathode structure whereby the other device components are covered by the mask and the cathode electrode is exposed through the opening in the mask;
  - forming an emitter on the cathode electrode portion exposed through the mask;
  - rotating the mask away from the cathode structure and the other device components;

rotating the cathode structure and the at least one other device component to an upright position; and locking the cathode structure and the at least one other device component in the upright position.

2. The process of claim 1, wherein the structural regions comprise silicon, and wherein the sacrificial regions comprise phosphosilicate glass.

3. The process of claim 1, wherein the one or more flexural members comprise one or more hinge mechanisms.

4. The process of claim 1, wherein the step of providing the structure comprises steps of providing a silicon wafer, forming a silicon nitride layer, forming and patterning the plurality of structural regions, and forming and patterning the plurality of sacrificial regions.

5. The process of claim 1, wherein the at least one other device component comprises a grid.

6. The process of claim 5, wherein the cathode electrode comprises cathode flexural members and the grid comprises a grid flexural members, and wherein the cathode flexural members and grid flexural members are attached to a device substrate.

7. A process for fabricating a vacuum microelectromechanical device comprising:

providing a device substrate comprising a cathode electrode, a grid, and an anode wherein the cathode, grid, and anode are each attached to the device substrate by one or more flexural members, wherein the cathode surface is substantially parallel to the substrate surface and a movable mask with an opening provided therein that is attached to the device substrate by one or more flexural members;

rotating the mask over the grid, the anode and an electrode portion of the cathode such that the cathode electrode surface is exposed through the mask opening;

35 forming electron emitters on the exposed cathode electrode surface to form a cathode;

rotating the mask away from the grid, the anode and the cathode; and

40 moving the cathode about the one or more cathode flexural members and moving the grid about the one or more grid flexural members and moving the anode about one or more anode flexural members such that the cathode surface and the grid surface and the anode surface are substantially parallel to each other and substantially perpendicular to the substrate; and

45 locking the cathode, grid and anode into position using locking mechanisms formed on the substrate.

8. The process of claim 7, wherein prior to the moving step the cathode electrode and the grid are substantially parallel to the surface of the device substrate, and wherein subsequent to the moving step the cathode electrode and the grid are substantially perpendicular to the device substrate surface.

9. The process of claim 7, wherein the cathode locking mechanism and the grid locking mechanism further comprise one or more locking flexural members, and wherein the process further comprises the step of securing the cathode and the grid in the substantially parallel relationship by moving the cathode locking mechanism into contact with the cathode and by moving the grid locking mechanism into contact with the grid.

10. The process of claim 9, wherein the one or more cathode flexural members comprise one or more hinges, wherein the one or more grid flexural members comprise one or more hinges, and wherein the one or more locking flexural members comprise one or more hinges.

11. The process of claim 7, wherein the step of forming electron emitters comprises forming carbon nanotubes on the cathode electrode surface.

12. The process of claim 11, wherein the step of forming electron emitters comprises:

forming a continuous or discontinuous catalyst layer on the cathode electrode surface; and

forming the carbon nanotubes on the catalyst layer by a chemical vapor deposition technique.

13. The process of claim 12, wherein the chemical vapor deposition technique is microwave plasma enhanced chemical vapor deposition.

14. The process of claim 11, wherein the step of forming electron emitters comprises:

spraying a mixture of the carbon nanotubes and a solvent onto the cathode electrode surface, and

performing an anneal.

15. The process of claim 7, wherein the step of providing the device substrate comprises steps of providing a silicon wafer, forming a silicon nitride layer, forming and patterning a plurality of silicon regions, forming and patterning a plurality of sacrificial regions, and treating the device substrate to remove the plurality of sacrificial regions.

16. The process of claim 7, wherein the surfaces of the cathode and the grid are  $10^6 \mu\text{m}^2$  or less.

17. The process of claim 7, wherein, after the moving step, the spacing between the cathode and the grid is less than 50  $\mu\text{m}$ .

30 18. A process for fabricating a plurality of vacuum microelectromechanical devices, comprising:

providing a substrate comprising a plurality of cathode electrodes attached to the device substrate by one or more cathode flexural members and having a cathode surface substantially parallel to the substrate surface, a plurality of grids attached to the device substrate by one or more grid flexural members, each cathode electrode having an associated grid, and one or more masks attached to the substrate with one or more flexural members, at least one mask having an opening therein, the plurality of cathode electrodes, the cathode flexural members, the plurality of grids and the grid flexural members being formed in structural regions formed on a substrate surface on and among sacrificial regions formed on the substrate;

35 rotating the one or more masks about its associated flexural members into place over portions of the device substrate such that the cathode electrode surfaces are exposed through the one or more mask openings and the grids are covered by the one or more masks;

forming electron emitters on the exposed cathode electrodes to form a plurality of cathodes;

rotating the one or more masks from over the cathodes and grids; and

40 moving each of the plurality of cathodes about the one or more cathode flexural members and moving each of the plurality of grids about the one or more grid flexural members such that the surface of each cathode and the surface of the associated grid are substantially parallel to each other and substantially perpendicular to the device substrate.

45 19. The process of claim 18, wherein at least a portion of the plurality of devices are interconnected to provide an integrated electronic circuit.

**11**

**20.** The process of claim **18**, wherein the step of forming electron emitters comprises forming carbon nanotubes on the cathode electrode surface.

**21.** The process of claim **20**, wherein the step of forming electron emitters comprises:

- forming a continuous or discontinuous catalyst layer on the surfaces of the cathode electrodes; and
- forming the carbon nanotubes on the catalyst layer by a chemical vapor deposition technique.

**22.** The process of claim **20**, wherein the step of forming electron emitters comprises:

**12**

spraying a mixture of the carbon nanotubes and a solvent onto the surfaces of the cathode electrodes, and performing an anneal.

**23.** The process of claim **18**, wherein the surfaces of the plurality of cathodes and the plurality of grids are  $10^6 \mu\text{m}^2$  or less.

**24.** The process of claim **18**, wherein, after the moving step, the spacing between each of the plurality of cathodes and each associated grid is less than  $50 \mu\text{m}$ .

\* \* \* \* \*